

# UNITED STATES PATENT OFFICE.

RUSSELL THAYER, OF PHILADELPHIA, PENNSYLVANIA.

## PROCESS FOR THE EXTRACTION OF PLATINUM AND SIMILAR METALS FROM THEIR SANDS AND ORES.

1,273,202.

Specification of Letters Patent.

Patented July 23, 1918.

No Drawing.

Application filed August 15, 1917. Serial No. 186,303.

*To all whom it may concern:*

Be it known that I, RUSSELL THAYER, of Philadelphia, in the county of Philadelphia and State of Pennsylvania, have invented 5 certain new and useful Improvements in Processes for the Extraction of Platinum and Similar Metals from Their Sands and Ores, whereof the following is a specification:

10 The invention is addressed to the recovery of the finely divided platinum, or similar metals, which may exist in such sands or ores initially in a free condition, or which may be released therein as the 15 result of fine grinding of the enveloping gangue.

I have discovered that notwithstanding the extremely high melting point of platinum and the rare metals of this group, and 20 their relatively high specific gravity, they can, when in an exceedingly comminuted condition, be volatilized under the effects of heat, and, by the use of a proper vehicle, can be carried away from the sands or ores 25 in which they are contained, and I have also discovered the further fact that the volatilized particles, when carried away, can be detained or suspended in water, so as to separate them from any vehicle which 30 may be employed as an adjunct in the volatilization.

I will now describe a preferred embodiment of my invention as applied to the recovery of platinum, it being understood that 35 I do not thereby restrict myself to the recovery of that particular metal alone.

I take a body of sand or ore of such cubic content as to be conveniently treated in a retort of reasonable size and preferably 40 grind the sands or ore very fine, say to about two hundred mesh. The degree of fineness of grinding will depend upon the character of the sands or ore and their metallic content. In many cases but slight grinding is 45 necessary, sufficient to release the metallic particles from the sands or rock particles. It will therefore be understood that the primary purpose of the grinding is not to reduce the size of the metallic particles 50 themselves, since ordinarily they occur in nature in an exceedingly comminuted condition, but is addressed mainly to their disengagement from the containing envelop.

I intimately mix with the sand or ore a 55 quantity of metallic mercury to which me-

tallic sodium has been added. This is preferably done during the grinding process, and water may be added, preferably to an extent just sufficient to thoroughly moisten the mass. As soon as the grinding and ad- 60 mixture of the mercury is complete, the magma is placed in a retort and heated sufficiently to cause the evaporation of the mercury by actual distillation. The dis- 65 charge from the retort is conducted into a body of water wherein the mercury is condensed and falls to the bottom. The ex- 70 ceedingly fine particles of platinum, how- 75 ever, notwithstanding the relatively high specific gravity of the metal itself, will re- 80 main suspended in the water for a consid- 85 erable time. Whether this phenomenon is due to some peculiar conditions of surface tension of the particles, or to some other factor characteristic of the conditions in 90 which they occur in sands and like bodies, I have not as yet definitely determined, but the suspension, or detention, of the plati- 95 num particles is so definite and so prolonged as to effectually separate them from the mercury particles, by which I believe them to have been in a certain sense conveyed in the act of volatilization. The treatment is continued until it becomes manifest that no more platinum is coming over. The water in which the particles from the retort have 100 been received, is then decanted from the mercury and is filtered, preferably by means of an ordinary paper filter.

The filter is then dried slowly and burned 90 in confinement, under such conditions as not to permit the carrying away of any of the finely divided platinum. The ash may then be treated with aqua regia, and the platinum recovered in any convenient way 95 from the resultant compound.

If desired, the mercury may be employed alone without the addition of sodium, or any other alkali metal may be employed in combination with the mercury together 100 with, or in place of, the sodium.

Having thus described my process in its preferred embodiment, I desire to state that I do not limit myself to the employment of a metallic vehicle as an adjunct to assist 105 in the volatilization, since I believe that to some extent the phenomenon will occur, even when aqueous vapor, or a gas, is properly employed as a vehicle or draft-producing current. I have found, however, that mer- 110

2  
 cury has a peculiar and valuable effect, in that while it does not, strictly speaking, form an alloy with platinum, it has a certain avidity therefor, which is manifested 5 by the actual picking up and temporary detention of platinum especially when finely divided by a body of mercury. This avidity appears to be greatly intensified when the mercury is combined with sodium or other 10 similar alkali metal and applied in the presence of water.

My belief is that under the circumstances above set forth, the mercury, when vaporized by distillation, carries along with it the 15 minute particles of platinum, which it has thus picked up, and I have described the phenomenon as "volatilization" of the platinum, in solid form, as distinguished from the change of physical condition which 20 would be implied by the term "vaporization."

Whatever may be the explanation, I have found it to be the fact that platinum can be thus separated and recovered from ore 25 in a manner available for commercial metallurgical practice, and I believe that my process can be made available for obtaining platinum from ores and sands, which heretofore have been considered not practically 30 useful as a source thereof. I believe that the phenomenon is characteristic of some of the so-called precious metals of the platinum group, such, for instance, as iridium, which is usually found in association with 35 platinum, and I therefore do not limit my claims to the recovery of platinum alone, but desire to comprehend the recovery of such other metals, which I term "similar," in the sense that they belong to the platinum 40 group, and while they have a high melting point and high specific gravity comparable to those of platinum, are capable of volatilization when in a finely divided form.

Having thus described my invention, I 45 claim:

1. The hereinbefore described process of recovering finely divided platinum and similar metals from sands or ore, which consists in volatilizing the finely divided metallic

particles by heat, at a temperature below 50 the melting point of the metal; carrying away the volatilized particles by a suitable vehicle; and collecting the volatilized particles.

2. The hereinbefore described process of 55 recovering finely divided platinum and similar metals from sands or ore, which consists in mixing the sands or ore with metallic mercury; subjecting the magma to a temperature sufficient to distil the mercury, but 60 below the melting point of the platinum or similar metal; collecting the distilled mercury and volatilized platinum or similar metal; and separating the platinum or similar metal from the mercury. 65

3. The hereinbefore described process of recovering finely divided platinum and similar metals from sands or ore, which consists in mixing the sands or ore with metallic mercury and an alkali metal; subjecting the 70 magma to a temperature sufficient to distil the mercury, but below the melting point of the platinum or similar metal; collecting the distilled mercury and volatilized platinum or similar metal; and separating the 75 platinum or similar metal from the mercury.

4. The hereinbefore described process of recovering finely divided platinum and similar metals from sands or ore, which consists 80 in mixing the sands or ore with metallic mercury; subjecting the magma to a temperature sufficient to distil the mercury, but below the melting point of the platinum or similar metal; collecting the mercury and 85 platinum or similar metal in water; separating the mercury; collecting the platinum or similar metal by filtration; and recovering the platinum or similar metal from the filter residuum. 90

In testimony whereof, I have hereunto signed my name at Philadelphia, Pa., sylvania, this eighth day of August, 1917.

RUSSELL THAYER.

Witnesses:

JAMES H. BELL,  
A. REID.

Copies of this patent may be obtained for five cents each, by addressing the "Commissioner of Patents, Washington, D. C."